

W. A. HALL.  
PROCESS OF MAKING MOTOR FUEL.  
APPLICATION FILED JAN. 23, 1915.

1,175,910.

Patented Mar. 14, 1916.



Witnesses.

N.J. Hayworth  
B. Heidenreich

Inventor.

William A. Hall - by

A. B. Foster  
his Attorney

# UNITED STATES PATENT OFFICE.

WILLIAM AUGUSTUS HALL, OF NEW YORK, N. Y.

## PROCESS OF MAKING MOTOR-FUEL.

1,175,910.

Specification of Letters Patent. Patented Mar. 14, 1916.

Application filed January 23, 1915. Serial No. 3,955.

*To all whom it may concern:*

Be it known that I, WILLIAM AUGUSTUS HALL, a citizen of the United States of America, and residing at New York city, New York, United States of America, have invented a certain new and useful Improvement in Processes of Making Motor-Fuel, of which the following is a specification.

This invention relates to the production of a new fuel suitable for use in automobile engines and possessing peculiar and highly valuable qualities not possessed by the ordinary gasolene of commerce. It is a slow burning fuel yet has an initial boiling point as low as gasolene and as large fractions volatile at low temperature say below 80° C. It is substantially free from liability to pre-ignite and therefore in an engine using the fuel, knocking does not occur even with the spark advanced, to so great an extent as with ordinary gasolene. As a direct result there is much less wear and tear on the engine, and the engine can be operated while under full load at lower engine speed or on a higher gear than when run on gasolene, which means a considerable saving in fuel consumption, less frequent changing of gears and slipping of clutches. Such fuel has been found particularly advantageous for use in commercial vehicles and in city traffic where frequent stopping and starting is required. This new fuel produced in the manner hereinafter described can be "cut" at a higher temperature than can a gasolene—it can be "cut" say at 180° C. as compared with 160° C. in the case of an ordinary gasolene. Its larger fractions volatile at low temperature have been found to carry complete combustion to the fractions volatile only at the highest temperatures, a considerably increased mileage per gallon consumed being the result.

The low flash point and low initial boiling point give in an engine run on the fuel, great ease in starting in cold weather, and owing to its large fractions volatile at low temperatures great flexibility and quickness of acceleration is obtained. It has been found that as great flexibility and ease of starting can be obtained with this fuel when "cut" at 180° C. and of specific gravity 0.760 as can be obtained on gasolene of specific gravity 0.730 "cut" at 160° C.

A distinguishing characteristic of the new

fuel is that it contains a proportion of unsaturated hydrocarbons which proportion will naturally vary with the oil used in its production. It contains a large percentage of hydrocarbons of the ethylene series but is nevertheless quite free from the objectionable features ordinarily inherent in products containing more than a small percentage of hydrocarbons of this series. The fuel having these peculiar and highly valuable properties is the direct result of an endothermic chemical reaction between a gas which would be permanent under ordinary conditions of temperature and pressure, and a vapor of a hydrocarbon spirit which vapor if condensed to a liquid in the customary manner at atmospheric temperature, would not answer the purpose of a satisfactory motor fuel, the combination of the permanent gas and vapor being effected by mechanical compression at a temperature sufficiently high to maintain the spirit portion under treatment, largely or wholly in the state of vapor. The process of production therefore has as its main feature the bringing about of this endothermic reaction the other stages being the production of the gas and vapor the bringing of them into the right condition for reaction and the treatment subsequent to the reaction to produce a refined spirit. The process thus consists of the following steps:

1. Cracking an oil—(which may be crude, "gas", fuel, lamp or almost any distillate that in itself has a range of boiling temperatures that would not permit its use as a fuel in the ordinary automobile engine)—in a continuous tube of small size, one to three inches, and of sufficient length, at an average temperature of from 540° C. to 600° C. on the exterior of the tube and under pressure preferably of about 75 lbs. per square inch, with a speed of flow of oil in the pipe regulated to produce a maximum of cracking with a minimum of fixed or permanent gas consistent with economy of operation.

2. Expanding the product subsequent to the cracking operation by reducing the pressure.

3. Cooling the vapors and gases when in this expanded state and from them separating fractions which have relatively high boiling points.

4. Producing an endothermic chemical reaction between the gases and vapors, by compressing the same, under substantially adiabatic conditions, in a mechanical compressor 5 to a pressure preferably from 100 to 125 lbs. per square inch together with all the gas that has been produced along with all the spirit vapors that boil below the point of "cut", admitting these into the cylinder of 10 the compressor at a temperature sufficiently high that they enter while in the shape of vapor and mist, the fixed gas that has not been attached being permitted to separate after cooling subsequent to the mechanical 15 compression and be collected for other use subsequent to compression. I use the term "adiabatic", in this specification in the same sense in which said term is defined in Hasting and Beach's *General Physics*, (published, Boston 1899) in which it is stated that "a body is said to undergo an adiabatic change when its condition is altered, without its gaining or losing heat to other bodies". In the process of the present invention, 20 I compress the gases and vapors, without materially adding to or taking away from the number of heat units present in the gases and vapors, by any influences outside the gases and vapors present. There may, 25 of course, be a small amount of heat radiated or otherwise lost from the surface of the compressor, to the outside atmosphere, but I do not purposely take away or add to the heat units. It is to be noted, that the endothermic reaction which takes place in the 30 gases themselves is not "gaining or losing heat to other bodies."

5. Clarifying and deodorizing the product by extracting the yellow resinous colloidal 40 matter which it contains, preferably by distilling it in the presence of a small amount of fullers' earth.

The accompanying drawing illustrates an 45 apparatus suitable for carrying out the process, up to the condensation of the motor fuel. The refining of the product may be performed in apparatus which is well known for the purpose and which it is not necessary to illustrate.

50 In the practice of this process I start with a crude oil or a distillate which may be a "gas oil" of about 0.860 specific gravity or a fuel oil of say 0.950 specific gravity or a low grade lamp oil of about 0.82 specific 55 gravity. In fact the process is adapted to almost any mineral oil and with very slight modifications of operation. This oil is pumped by means of a pump 1 through a coil of 1" or 1½" pipe 2 located above a furnace 3 where it is pre-heated by the hot products of combustion arising from the furnace 3. It is then passed through the coil of pipe 4 heated by the burners 5 to an average temperature of from 540° C. to 600° 60 C. according to the oil used, the temperature

being determined by a pyrometer 6, the thermo-couple of which is placed in the center of the nest of tubes 4. The temperature of the gases and vapors inclosed in the tubes may be of somewhat lower temperature than that existing at the exterior of the tube, opposite the same point, varying with the speed of flow of the fluid in the coil and slightly higher at the bottom of the bends and slightly lower at the top. As an example, the oil is pumped through this coil of tubes at about the rate of 50 to 70 gallons per hour which rate will be varied with the quality of the oil used. The length of tubing of coil 4 is about 320 feet. The rate of flow and the length of coil mentioned are simply given as examples of rate and length producing good results; the rate of flow may be increased or reduced by quite a considerable amount without greatly changing the result. The coil may be increased in length but if of 1" pipe could not be reduced much below the figure mentioned without changing the result. The coil 4 may be heated with a flame of gas or by the combustion of oil, coal or coke, or in any other suitable manner. In the coil 4, the oil is partially cracked and there is produced a considerable amount of gas which would remain as permanent gas under ordinary conditions. 95 From coil 4 the gases and cracked oil in the state of vapor pass in the direction of the arrow through pipe 7 which is fitted with a valve 8. This valve 8 is used as the main throttle and governs the amount of oil passing through coil 4 and also governs the pressure maintained in said coil. A pressure of about 75 lbs. per square inch maintained in coil 4 appears to give the best results. After passing the valve 8 the gases are permitted to expand into the dephlegmator 9 fitted with an air jacket 10 and preferably filled with short pieces of pipe or kindred shapes or the like 11 wherein the pressure is decreased from 75 lbs. per square inch (the pressure 110 within the coil 4) down to about 10 lbs. per square inch or less and the temperature is reduced down to about 325° C. Carbon is thrown out in large quantities by the expansion of the gases and collects on the filling 115 material in this and the succeeding dephlegmator.

The portions of oil not volatile at the temperature of about 325° C. condense in dephlegmator 9 and are extracted from the bottom by way of a pipe 12 in the form of a so called "heavy residue" of a gravity of about 1.0. The more volatile portions pass on through pipe 13 in the direction of the arrow and through a similar dephlegmator 14 where the temperature is reduced to the point where it is desired to make the final "cut", usually about 180° C., the condensable portion being extracted by way of a pipe 15 from the bottom of the dephlegmator 14, 130

said residue being termed "light residue." This residue is usually of a gravity of about 0.880 and is used as raw material for a second run through the cracking coil 4. The 5 portion volatile at the temperature of the cut (for example 180° C.) accompanied by all of the gas is then passed through a separating tank 16, (from which any liquid may return by pipe 16' to dephlegmator 14) or 10 may be otherwise utilized then at its full temperature (that is to say, without any material amount of further cooling) or as near to it as possible the vapors and gases are passed through the cylinder of a mechanical compressor 17 in which the pressure is raised, preferably up to 100 or 125 lbs. per square inch. In the cylinder of this compressor there is produced between the products an endothermic reaction, which is 15 shown by a decrease in temperature at the exit as compared with the inlet or at any rate by a much less increase in temperature than would occur provided no endothermic chemical action took place therein. The 20 product is then passed by way of a pipe 18 to coolers, 19, 20 and thence to a receiver 21, where the liquid collects, and the uncondensed gas finds exit through the pipe 22.

The new product is quite stable and of a 25 yellow color and has a disagreeable varnish-like odor, and contains a material, which upon evaporation of the liquid, remains as a dark orange, non-drying substance, with a strong varnish-like odor. This product 30 accordingly could not well be used as a successful automobile fuel. It is therefore now clarified and rendered water white and its disagreeable odor removed by redistillation without the loss of its large fractions boiling 35 at low temperature and without any substantial change in its specific gravity. This is effected by agitating the spirit with, say about 10% of its weight of fullers' earth or equivalent mineral matter, separating the spirit from the mineral matter 40 and distilling it. I find that although this agitation removes very little of the color (judging by appearances), when distilled the distillate is water white. The coloration 45 and odor may be removed by direct distillation of the spirit from a mixture with fullers' earth or the like or the clarifying of this crude yellow spirit may be effected by treatment with a small amount of sulfuric acid or otherwise.

The step of cooling the gases and vapors produced by cracking oil, while at a pressure materially below that of cracking is not claimed herein, but is claimed in my 50 copending application 852,965 filed July 24, 1914.

The cracking of oil at relatively high temperatures, removing materials having boiling points too high for the production 55 of motor fuel and the subsequent cooling

and condensation of motor fuel from the remaining gases and vapors is broadly claimed in my copending applications 824,194 filed March 12, 1914, and 829,634, filed April 4, 1914.

The crude and refined products produced in accordance with the present process and certain modifications thereof are claimed in my copending applications 26,395, filed May 6, 1915, and 26,546 filed May 7, 1915.

The apparatus shown and described herein is claimed in my copending application 77,357, filed February 9, 1916.

Having described my invention, what I claim and desire to secure by Letters Patent of the United States is:

1. The process of forming volatile hydrocarbons, liquid at ordinary temperatures, by subjecting the gases and vapors resulting from the cracking and gasifying of hydrocarbon oils to so great an increase of pressure under substantially adiabatic conditions while the gases and vapors are in a heated state as to produce an endothermic reaction therein, and subsequently condensing the products so formed.

2. Process of producing from mineral oil, liquid fuel suitable for use in automobile engines consisting in subjecting the gases and vapors resulting from the cracking and gasifying of mineral oil to sudden increase of pressure sufficient to produce an endothermic reaction therein, while the gases and vapors are in a heated state, and subsequently condensing the products so formed.

3. Process of producing from mineral oil, liquid fuel suitable for use in automobile engines, consisting in cracking the oil under pressure materially above atmospheric to produce gases and vapors, expanding such gases and vapors, then subjecting such gases and vapors to sudden increase of pressure while the gases are in a heated state, condensing the products so formed and redistilling with mineral matter of the fullers' earth type.

4. Process of producing from mineral oil, liquid fuel suitable for use in automobile engines, consisting in cracking the oil under pressure to produce gases and vapors, expanding such gases and vapors, then subjecting such gases and vapors to sudden increase of pressure sufficient in amount to produce an endothermic reaction therein, while the gases are in a heated state, condensing the products so formed and clarifying the product.

5. Process of producing from mineral oil a liquid fuel suitable for use in automobile engines consisting in cracking an oil under pressure at a high temperature to produce gases and vapors, releasing the pressure of the gases and vapors produced within a short time after their production, passing such gases and vapors through a mass of ma-

4

terial capable of removing solid materials, and materials having high boiling points, partially cooling the gases and vapors to remove the fractions of high boiling from those of low boiling points, mechanically compressing the partially cooled, but still warm vapors and gas from which the fractions of high boiling points have been separated to attach portions of the gas to the vapors, cooling and condensing the products resulting from the compression under substantially the pressure of compression thereby forming a liquid, removing the portions of gas not affixed to vapor on compression and condensation, and clarifying and deodorizing the liquid product.

6. Process of producing from mineral oil a liquid fuel suitable for use in automobile engines consisting in cracking an oil at a high temperature under pressure to produce gases and vapors, expanding the gases and vapors to deposit solid matter carried by the gases, partially cooling the gases and vapors to remove the fractions boiling at high points, from those boiling at low points mechanically compressing the hot vapors and gas from which the fractions boiling at high points have been extracted to attach portions of the gas to the vapors formed, cooling and condensing the products resulting from the compression under substantially the pressure of compression thereby forming a liquid, removing the portions of gas not affixed to vapor during the compression and condensation and clarifying and deodorizing the liquid product.

7. Process of producing from mineral oil a liquid fuel suitable for use in automobile engines consisting in cracking an oil at a high temperature under pressure to produce gases and vapors, releasing the pressure of the gases and vapors produced immediately subsequent to their production, passing the gases and vapors through a dephlegmator to remove the fractions boiling at high points from those boiling at low points, mechanically compressing the warm vapors and gas from which the fractions boiling at high points have been extracted to attach portions of the gas to the vapor formed, cooling and condensing the products resulting from the compression under substantially the pressure of compression thereby forming a liquid, removing the portions of gas not affixed to vapor on compression and condensation, and clarifying and deodorizing the liquid product.

8. Process of producing from mineral oil a liquid fuel suitable for use in automobile engines consisting in cracking an oil under a pressure of about 70 lbs. per square inch, at a temperature of from about 540° C. to 600° C. to produce gases and vapors, releasing the pressure of the gases and vapors produced

immediately subsequent to their production, passing such gases and vapors through a material on which any free carbon carried by the gases will deposit, partially condensing the gases and vapors to remove the fractions boiling at high points from those boiling at low points, mechanically compressing the portions boiling at the lower temperature along with the gas to a pressure of not less than about 125 lbs. per square inch the hot vapors and gas from which the fractions boiling at high points have been extracted, to attach portions of the gas to the vapor formed, cooling and condensing the products resulting from the compression under substantially the pressure of compression whereby to form a liquid, removing the portions of gas not chemically affixed to vapor on compression and condensation, and clarifying and deodorizing the liquid product.

9. Process of producing from mineral oil a liquid fuel suitable for use in automobile engines consisting in subjecting the oil to a high temperature and a moderate pressure to produce cracking, extracting the high boiling point fractions from the cracked products, compressing the remainder of the product while in the vapor and gaseous state sufficiently to produce an endothermic reaction between such gas and vapor, and clarifying and deodorizing the product by distillation with mineral matter.

10. In the cracking of oil and the production of motor spirit therefrom, the step of subjecting the warm vapors and gases to a sufficient increase of pressure to effect a lowering of temperature therein.

11. The step of producing, by substantially adiabatic compression of the gases and vapors produced by cracking oils an endothermic chemical reaction therein.

12. In the process of producing motor fuel from hydrocarbon oils, the step of cracking the oils, and thereafter subjecting at least a portion of the gases and vapors produced therefrom, to a sufficient increase in pressure, to produce an endothermic chemical reaction therein.

13. A process of producing from mineral oil, a liquid fuel suitable for use in internal combustion engines, consisting in cracking the oil under pressure to produce gases and vapors, expanding said gases and vapors and thereafter subjecting said gases and vapors to an increase in pressure, sufficient to produce an endothermic reaction therein.

14. A process of producing from mineral oil, a liquid fuel suitable for use in automobile engines, which comprises cracking mineral oil under pressure to produce gases, light vapors and heavy vapors, partially cooling said gases and vapors, and thereafter subjecting the uncondensed portion thereof to an increase in pressure sufficient

to produce an endothermic reaction in said gases and vapors.

15. In the manufacture of motor fuel the step of adiabatically compressing a mixture of hydrocarbon vapors and gases sufficiently to produce an endothermic chemical reaction therein.

16. A process of forming volatile hydrocarbons, which comprises subjecting the 10 gases and vapors resulting from the cracking and gasifying of hydrocarbon oils, to so great an increase of pressure, without heating or cooling the said gases and vapors from the outside, to any substantial amount, 15 and while the gases and vapors are in a heated state, as to produce an endothermic

reaction therein, and subsequently condensing the products so formed.

17. In the production of motor fuel, the step of subjecting gases and vapors produced by cracking oils, to so great an increase of pressure while at a temperature materially below 325° C., as to produce an endothermic reaction therein.

In testimony whereof I have signed my 25 name to this specification in the presence of two subscribing witnesses.

WILLIAM AUGUSTUS HALL.

Witnesses:

R. WILLIAMS,  
H. D. JAMESON